# EUROPEAN PATENT SPECIFICATION

(11) **EP 4 079 172 B1**
(45) Date of publication and mention of the grant of the patent: **15.07.2026**
(21) Application number: 20902306.8
(22) Date of filing: 13.10.2020
(51) Int. Cl.: A24F 40/46, A24F 40/70, H05B 3/10, H05B 3/34, H05B 3/36, H05B 3/42, A24F 40/20

(54) **FLEXIBLE HEATING ASSEMBLY AND FABRICATION METHOD THEREOF**
BIEGSAME HEIZANORDNUNG UND DAZUGEHÖRIGES HERSTELLUNGSVERFAHREN
ENSEMBLE CHAUFFANT FLEXIBLE ET PROCÉDÉ DE FABRICATION ASSOCIÉ

(30) Priority: 20.12.2019 CN 201911327773
(43) Date of publication of application: 26.10.2022
(73) Proprietor: Shenzhen Smoore Technology Limited, Shenzhen, Guangdong 518102 (CN)
(72) Inventor: ZHOU, Hongming, Shenzhen, Guangdong 518102 (CN); CHENG, Zhenqian, Shenzhen, Guangdong 518102 (CN); XIAO, Junjie, Shenzhen, Guangdong 518102 (CN)
(74) Representative: Westphal, Mussgnug & Partner, Patentanwälte mbB
(86) International application number: PCT/CN2020/120691
(87) International publication number: WO 2021/120802

(56) References cited:
- WO-A1-2016/184978
- CN-A- 106 028 486
- CN-A- 106 579 564
- CN-A- 106 579 564
- CN-A- 108 513 378
- CN-A- 109 527 660
- CN-A- 110 495 642
- CN-A- 111 053 298
- CN-U- 206 923 677
- CN-U- 209 376 696
- CN-U- 209 769 004
- US-A- 5 369 723
- US-A- 5 408 574
- US-A1- 2018 093 455

## Description

### FIELD

The present invention relates to the field of vaporization, and more specifically, to a flexible heating assembly and a fabrication method thereof.

### BACKGROUND

As a new type of electronic cigarette, a heat not burn cigarette mainly heats tobacco by accurately controlling a temperature after a heating element is energized, and can quickly release tobacco extracts in the tobacco under a low temperature condition, so that a consumer can have a smoking experience similar to that of conventional tobacco-burning cigarettes but with less harmful components being released. Currently, different types of heating bodies are launched at home and abroad to heat an aerosol-generating substrate such as tobacco. The heating bodies are, for example, a sheet-shaped heating element, a rod-shaped heating element, and a tubular heating element.

A principle of heating tobacco by the sheet-shaped heating element and rod-shaped heating element is that a heating sheet is inserted into a middle part of the cigarette, and after being energized, a resistance material on a surface of the heating sheet radiates heat to heat the tobacco and conducts the heat in the tobacco. According to this heating manner, the tobacco can be only inhaled after being preheated for a period of time (usually 15s to 20s) to fully heat the tobacco. Due to a small heating area, the amount of vapor is small (compared with a real cigarette) after the tobacco is baked. In addition, because the tobacco closest to the heating sheet is over-baked after a plurality of times of inhaling, a burnt taste occurs in the later stage of inhaling, and the taste consistency is poor.

A principle of heating tobacco by the tubular heating element is that a cigarette is inserted into a tube, and a resistance material on a wall surface of the tube radiates heat after being energized to heat the tobacco in the tube and conducts the heat in the tobacco. Theoretically, according to this heating manner, a contact area between the tobacco and the heating element can be increased, and a preheating time of the tobacco is shortened, so that vapor can be generated quickly. However, due to a gap between an inner wall of the tube and the cigarette, the heat conduction is slow, resulting in a long preheating time and a small amount of vapor in the early stage of heating.

Therefore, a heating element is urgently required that can quickly and fully heat the aerosol-generating substrate and generate a large amount of vapor through baking.

Publications CN 108 513 378 A, US 2018/093455 A1, US 5 408 574 A and WO 2016/184978 A1 are considered to be relevant to the present application. In particular, US 5 408 574 A discloses a heater having a ceramic substrate 1 and resistive heating elements 2. The substrate 1 provides physical support for resistive heating elements 2. The ceramic substrate 1, while being rigid enough to physically support the resistive heating elements 2, can also be made flexible enough to facilitate easy handling and resist fracture during the manufacturing process. A tobacco flavor-generating medium may be sprayed onto the heating elements and subsequently dried before use. The resistive and conductive layers can be applied to the substrate in several ways, including techniques such as sputtering, physical vapor deposition, chemical vapor deposition, thermal spraying, and DC magnetron sputtering.

### SUMMARY

A technical problem to be solved by the present invention is to provide a flexible heating assembly and a fabrication method thereof for the foregoing defects in the related art. The problem underlying the present application is solved by a flexible heating assembly having the features of claim 1 and by a method for fabricating a flexible heating assembly having the features of claim 8.

The technical solution adopted by the present invention to solve the technical problem is to construct a flexible heating assembly according to claim 1.

In some embodiments, the conductive circuits, and the flexible protective film are all formed by magnetron sputtering coating.

In some embodiments, the sheet-shaped flexible substrate includes at least one of aluminosilicate fiber paper, PI film, and casting ceramic sheet.

In some embodiments, the flexible protective film includes at least one of casting sheet, nitride ceramic material, and oxide ceramic material, and the thermal expansion coefficient of the flexible protective film adapts to the thermal expansion coefficient of the sheet-shaped flexible substrate.

In some embodiments, the flexible protective film includes at least one of ZrO₂ composite film, Al₂O₃ composite film, SiO₂ composite film, and Si₃N₄ composite film prepared through direct current magnetron sputtering or radio frequency magnetron sputtering, and the thickness of the flexible protective film is from 100 nm to 1000 nm.

In some embodiments, the thickness of the at least one heating circuit is from 1 µm to 3.5 µm, and the thickness of the conductive circuits is from 1 µm to 5 µm.

In some embodiments, the heating element further includes electrode leads respectively connected to the conductive circuits.

In some embodiments, the at least one heating circuit includes a transition layer disposed on the sheet-shaped flexible substrate and a heating layer disposed on the transition layer.

In some embodiments, the transition layer includes at least one of Cr, ZrNi, and TiN, and the heating layer includes at least one of Pt, AgPd, AuPd, PtRu, PtRh, NiCr, and NiCrAlY.

In some embodiments, the conductive circuits include a bottom layer disposed on the sheet-shaped flexible substrate, an intermediate buffer layer disposed on the bottom layer, and a conductive layer disposed on the intermediate buffer layer.

In some embodiments, the bottom layer includes at least one of pure Ti or pure Ni, the intermediate buffer layer includes at least one of pure Ti and pure Ni, and the conductive layer includes at least one of Au, Ag, and Cu.

The present invention further provides a method for fabricating a flexible heating assembly according to claim 8.

In some embodiments, the method further includes: in step S1, wiping and cleaning the sheet-shaped flexible substrate with alcohol, placing the sheet-shaped flexible substrate in a coating machine cavity, vacuuming and preheating the coating machine cavity, and ion-cleaning the surface of the sheet-shaped flexible substrate; and

in step S4, introducing argon and oxygen in a ratio of 1:1 into the coating machine cavity until the working air pressure therein reaches 0.4 Pa; turning on a first power supply for a SiO₂ target, a ZrO₂ target, an Al₂O₃ target, or a Si₃N₄ target; and performing magnetron sputtering at a power density between 2 W/cm² and 6 W/cm² and at a temperature between room temperature and 500°C to form the protective film with a thickness between 100 nm and 1000 nm.

In some embodiments, step S2 includes:
performing magnetron sputtering on the sheet-shaped flexible substrate to form a transition layer; and
performing magnetron sputtering on the transition layer to form a heating layer.

In some embodiments, the method further includes: in step S2, introducing argon into the coating machine cavity until the working air pressure therein reaches 0.5 Pa, turning on a second power supply for a Cr target, a ZrNi target, or a TiN target, coating a first film on the sheet-shaped flexible substrate for 5 minutes to 15 minutes at a power density between 6 W/cm² and 8 W/cm² and at room temperature to form the transition layer with a thickness between 10 nm and 200 nm, and
turning off the second power supply for the Cr target, the ZrNi target, or the TiN target, turning on a third power supply for a NiCr target, a NiCrAlY target, a Pt target, an AgPd target, an AuPd target, a PtRu target, or a PtRh target, and coating a second film on the transition layer for 60 minutes to 120 minutes at a power density between 6 W/cm² and 8 W/cm² and at room temperature to form the heating layer with a thickness between 1 µm and 2.5 µm.

In some embodiments, step S3 includes:
performing magnetron sputtering on the sheet-shaped flexible substrate to form a bottom layer;
performing magnetron sputtering on the bottom layer to form an intermediate buffer layer;
performing magnetron sputtering on the intermediate buffer layer to form a conductive layer; and
soldering an electrode lead on the conductive layer to form a conductive electrode.

**In** some embodiments, the method further includes: in step S2, introducing argon into the coating machine cavity until the working air pressure therein reaches 0.5 Pa; turning on a fourth power supply for a Titanium target or a Nickel target; coating a third film on the sheet-shaped flexible substrate for 5 minutes to 10 minutes at a power density between 6 W/cm² and 8 W/cm² and at room temperature to form the bottom layer;
turning off the fourth power supply for the Titanium target or the Nickel target; turning on a fifth power supply for a Nickel target or a Titanium target; coating a fourth film on the bottom layer for 10 minutes to 30 minutes at a power density between 6 W/cm² and 8 W/cm² and at room temperature to form the intermediate buffer layer; and
turning off the fifth power supply for the Nickel target or the Titanium target; turning on a sixth power supply for a silver target, a copper target, or a gold target; and coating a fifth film on the intermediate buffer layer for 30 minutes to 120 minutes at a power density between 4 W/cm² and to 8 W/cm² and at room temperature to form the conductive layer.

According to the present invention, the heating assembly is in spiral cylindrical shape, and the heating assembly includes the heating element according to any one of the above and an aerosol-generating substrate coated on the side surface of the heating element on which the at least one heating circuit is disposed.

The aerosol-generating substrate includes a viscous substance, and the thickness of the aerosol-generating substrate may be from 0.5 mm to 1 mm.

There is also provided an aerosol generator, including the heating element according to any one of the above.

Implementing the present invention at least has the following beneficial effects: when the flexible heating element is in use, an aerosol-generating substrate is coated on the side surface of the heating element, on which the at least one heating circuit is disposed, and then the heating element coated with the aerosol-generating substrate is wound into a shape of a spiral cylinder to form a heating assembly. This structure can increase a direct contact area and a heating area between the heating element and the aerosol-generating substrate. The heating element can heat the aerosol-generating substrate in all directions, and the aerosol-generating substrate is heated faster and more uniformly, which reduces a preheating time, so that the heating element can reach an instant inhaling mode, which has advantages such as fast vapor generation and a large amount of vapor.

### BRIEF DESCRIPTION OF THE DRAWINGS

The present invention is further described below with reference to accompanying drawings and embodiments, and in the accompanying drawings:
FIG. 1 is a fabrication flowchart of a heating assembly according to some embodiments of the present invention;
FIG. 2 is a schematic structural diagram of a heating circuit of a heating element according to some embodiments of the present invention; and
FIG. 3 is a schematic structural diagram of a conductive circuit of a heating element according to some embodiments of the present invention.

### DETAILED DESCRIPTION

To provide a clearer understanding of the technical features, objectives, and effects of the present invention, specific implementations of the present invention are described with reference to the accompanying drawings.

As shown in FIG. 1 to FIG. 3, the flexible heating assembly in some embodiments of the present invention includes a flexible heating element 1 and an aerosol-generating substrate 2 coated on a side surface of the heating element 1. The flexible heating element 1 includes a sheet-shaped flexible substrate 11, at least one heating circuit 12 disposed on the substrate 11, conductive circuits 13 disposed on the substrate 11 and respectively connected to two ends of the heating circuit 12, electrode leads 14 respectively connected to the conductive circuits 13, and a flexible protective film covering the at least one heating circuit 12.

When the flexible heating element 1 is in use, an aerosol-generating substrate 2 added with a viscous substance (for example, reconstituted tobacco added with a viscous substance) can be coated on the side surface of the heating element 1 on which the heating circuit 12 is disposed, and the thickness of the aerosol-generating substrate 2 may be from 0.5 nm to 1 mm. Then the heating element 1 covered with the aerosol-generating substrate 2 is wound into a shape of a spiral cylinder to form a flexible heating assembly. This structure can increase the direct contact area and the heating area between the heating element 1 and the aerosol-generating substrate 2. The heating element 1 can heat the aerosol-generating substrate 2 in all directions, and the aerosol-generating substrate 2 is heated faster and more uniformly, which reduces a preheating time, so that the heating element 1 can reach an instant inhaling mode, which has advantages such as fast vapor generation and a large amount of vapor.

Two or more heating circuits 12 may be disposed on the substrate 11 of the heating element 1, and two ends of each heating circuit 12 are respectively electrically connected to the electrode leads 14. The aerosol-generating substrate 2 can be heated by segments, so that the aerosol-generating substrate 2 can be heated sequentially by segments instead of being heated at one time, which improves the utilization of the aerosol-generating substrate and the inhaling convenience, and simultaneously can avoid a burnt smell produced by over-baking the baked aerosol-generating substrate, thereby improving the inhaling taste. Each heating circuit 12 can be distributed in the axial direction of the substrate 11 after winding (the width direction of the substrate 11 in this embodiment), or can be distributed in a circumferential direction after winding (a length direction of the substrate 11 in this embodiment), or can be distributed in the axial and circumferential directions of the substrate 11 after winding.

To ensure the uniformity of the temperature field in a heating region, the heating circuit 12 needs to be formed into a proper pattern, such as an S shape, a spiral shape, a wave shape, or the like. A pattern of the heating circuit 12 may be prepared by using a mask method or an ion etching method. The mask method is to form the pattern of the heating circuit 12 on the substrate 11 after sputtering the heating circuit 12 by masking a non-patterned position on the substrate 11. The ion etching method is to first plate the heating circuit 12 on a whole surface of the substrate 11, after photoresist is applied for exposure and curing, ion-etch the exposed photoresist and a region of the heating circuit 12, and then remove the unexposed photoresist to form a required pattern of the heating circuit 12. A pattern of the conductive circuit 13 may also be prepared by using the mask method or the ion etching method.

The heating circuit 12, the conductive circuit 13, and the protective film can be all formed by magnetron sputtering coating. A manner of magnetron sputtering can reduce the overall thickness of the heating element 1, and simultaneously can improve the resistance consistency of the pattern of the heating circuit 12 and reduce a fluctuation range of TCR, which is more conducive to precise temperature control of the heating field.

The substrate 11 can be a transparent or non-transparent flexible insulating sheet with high temperature resistance, corrosion resistance, and a stable material structure, and provide a carrier for the sputtered heating circuit 12 and the conductive circuit 13. In some embodiments, the substrate 11 may be made of at least one of high-temperature-resistant flexible insulating polyimide film (namely, PI film), aluminosilicate fiber paper, and flexible ceramic sheet prepared by casting. The thickness of the substrate 11 may be from 0.5 mm to 2 mm.

A function of the heating circuit 12 is to stably generate heat after being energized, and to heat an aerosol-generating substrate, which can usually be made of a metal material with high resistivity (that is, high resistance) and more generated heat. In some embodiments, the heating circuit 12 may be formed by sputtering a metal or an alloy material, such as Pt, AgPd, NiCr, or NiCrAlY, on the transition layer after direct current or radio frequency magnetron sputtering is performed on the transition layer, and the thickness of the heating circuit 12 may be from 1 µm to 3.5 µm.

In some embodiments, the heating circuit 12 includes a transition layer 121 disposed on the substrate 11 and a heating layer 122 disposed on the transition layer 121. The transition layer 121 mainly enhances the bonding force between the heating layer 122 and the substrate 11, increases the structural stability, prevents separation, and improves the bonding stability between a film and a substrate when the heating element generates heat circularly. The transition layer 121 may be made of an alloy that forms a stable chemical bond with both the substrate 11 and the heating layer 122, for example, the transition layer 121 may be made of at least one of Cr, ZrNi, and TiN. The heating layer 122 should be made of a material with high resistivity, more generated heat, stable material structure performance after high temperature heating, and good high temperature oxidation resistance and corrosion resistance, for example, a precious metal material such as Pt, or a precious metal alloy material such as AuPd, PtRu, PtRh, or AgPd, or a high-temperature-resistant alloy material such as NiCr or NiCrAlY.

One end of the conductive circuit 13 is connected to the heating circuit 12, and the other end is connected to the electrode lead 14 to be welded with the electrode lead 14 and supply power to the heating circuit 12. The conductive circuit 13 has low resistivity (that is, low resistance), and generates few heat. In some embodiments, the conductive circuit 13 may be formed by sputtering a thin film, such as an Ag thin film, an Au thin film, or a Cu thin film after performing direct current or radio frequency sputtering pure Ti or Pure Ni, or plating the pure Ti and the pure Ni on the substrate. The thickness of the conductive circuit 13 may be equal to or slightly higher than the thickness of the heating circuit 12. In some embodiments, the thickness of the conductive circuit 13 may be from 1 µm to 5 µm.

In some embodiments, the conductive circuit 13 may include a bottom layer 131 disposed on the substrate 11, an intermediate buffer layer 132 disposed on the bottom layer 131, and a conductive layer 133 disposed on the intermediate buffer layer 132. The bottom layer 131 and the intermediate buffer layer 132 may respectively be made of at least one of pure Ti and pure Ni. The bottom layer 131 and the intermediate buffer layer 132 are respectively formed by coating, which helps form a certain thickness, and can further increase the structural stability and prevent separation. The conductive layer 133 may be made of a metal material with good stability and conductivity, for example, the conductive layer 133 may be made of at least one of Au, Ag, Ni, and Cu. Generally, silver or copper may be used due to low costs.

A function of the protective film is to reduce the erosive effect of oxygen and impurities on the heating circuit 12, prevent the heating circuit 12 from reacting with the aerosol-generating substrate 2 during heating, and reduce an impact of the accumulation of soot on the inhaling taste. Part regions of the conductive circuit 13 and regions on the substrate 11 where the conductive circuit 13 and the heating circuit 12 are not disposed may also be covered with a protective film. Because the conductive circuit 13 needs to be welded with the electrode lead 14, a region where the conductive circuit 13 is welded with the electrode lead 14 is not covered by the protective film. In some embodiments, the protective film may be a ceramic material with good flexibility, a thermal expansion coefficient adapting to the substrate 11, good high temperature stability, easy to clean, and good corrosion resistance, for example, a material such as casting sheet or Si₃N₄, or an oxide material such as ZrO₂, Al₂O₃, or SiO₂. The protective film may be prepared by at least one of ZrO₂ composite film, Al₂O₃ composite film, SiO₂ composite film, and Si₃N₄ composite film prepared through direct current or radio frequency magnetron sputtering, and the thickness of the protective film is from 100 nm to 1000 nm.

The present invention further provides a fabrication method for a flexible heating element, including the following steps:
S1: Processing before coating:
   a sheet-shape flexible substrate 11 is provided, after the substrate 11 is wiped and cleaned with alcohol, the substrate 11 is placed into a coating machine cavity, the coating machine cavity is vacuumized and preheated, and the surface of the substrate 11 is ion-cleaned.
S2: Formation of the heating circuit 12:
   Magnetron sputtering is performed on the substrate 11 to form the heating circuit 12.

Specifically, step S2 may include:
introducing argon until the working air pressure in the cavity reaches 0.5 Pa, turning on a Cr target power supply, and coating a film on the substrate 11 for 5 minutes to 15 minutes at a power density of from 6 W/cm² to 8 W/cm² and at a room temperature to form the transition layer 121 with a thickness of from 10 nm to 200 nm; and
then turning off the Cr target power supply, turning on a NiCr target power supply, and coating a film on the transition layer 121 for 60 minutes to 120 minutes at a power density of from 6 W/cm² to 8 W/cm² and at a room temperature to form the heating layer 122 with a thickness of from 1 µm to 2.5 µm.

S3: Formation of the conductive circuit 13:
Magnetron sputtering is performed on the substrate 11 to form the conductive circuit 13.

Specifically, step S3 may include:
introducing argon until a working air pressure in the cavity is 0.5 Pa, turning on of a Titanium target power supply, and coating a film on the substrate 11 for 5 minutes to 10 minutes at a power density of from 6 W/cm² to 8 W/cm² and at a room temperature to form the bottom layer 131; turning off the Titanium target power supply;
then turning on the Titanium target power supply, and coating a film 131 on the bottom layer for 10 minutes to 30 minutes at the power density of from 6 W/cm² to 8 W/cm² and at a room temperature to form the intermediate buffer layer 132; turning off the power supply of the Titanium target;
then turning on a silver target power supply, and coating a film on the intermediate buffer layer 132 for 30 minutes to 120 minutes at a power density of from 4 W/cm² to 8 W/cm² and at a room temperature to form the conductive layer 133; and
soldering an electrode lead 14 on the conductive layer 133 to form a conductive electrode.

S4: Formation of the protective film:
Argon and oxygen in a ratio of 1:1 are introduced until the working air pressure in the cavity reaches 0.4 Pa, and sputtering is performed at a sputtering power density of a direct current SiO₂ target power supply between 2 W/cm² and 6 W/cm² and at a temperature between room temperature and 500°C to form the protective film with a thickness of from 100 nm to 1000 nm.

There is provided an aerosol generator, including a cavity for accommodating a heating assembly and a heating assembly disposed in the cavity, wherein the heating element 1 of the heating assembly, after being energized and heated up, bakes and heats the aerosol-generating substrate 2 for the user to inhale.

While the invention has been illustrated and described in detail in the drawings and foregoing description, such illustration and description are to be considered illustrative or exemplary and not restrictive. It will be understood that changes and modifications may be made by those of ordinary skill within the scope of the following claims.

The terms used in the claims should be construed to have the broadest reasonable interpretation consistent with the foregoing description. For example, the use of the article "a" or "the" in introducing an element should not be interpreted as being exclusive of a plurality of elements. Likewise, the recitation of "or" should be interpreted as being inclusive, such that the recitation of "A or B" is not exclusive of "A and B," unless it is clear from the context or the foregoing description that only one of A and B is intended. Further, the recitation of "at least one of A, B and C" should be interpreted as one or more of a group of elements consisting of A, B and C, and should not be interpreted as requiring at least one of each of the listed elements A, B and C, regardless of whether A, B and C are related as categories or otherwise. Moreover, the recitation of "A, B and/or C" or "at least one of A, B and C" should be interpreted as including any singular entity from the listed elements, e.g., A, any subset from the listed elements, e.g., A and B, or the entire list of elements A, B and C.

## Claims

1. A flexible heating assembly, comprising:
a heating element, comprising:
a sheet-shaped flexible substrate (11);
at least one heating circuit (12);
conductive circuits (13); and
a flexible protective film;
wherein the at least one heating circuit (12) is disposed on the sheet-shaped flexible substrate (11), the conductive circuits (13) are disposed on the sheet-shaped flexible substrate (11) and respectively connected to the ends of the at least one heating circuit (12), and the flexible protective film covers the at least one heating circuit (12); and
an aerosol-generating substrate comprising a viscous substance;
wherein the aerosol-generating substrate is coated on the side surface of the heating element, on which the at least one heating circuit (12) is disposed, and the heating element coated with the aerosol-generating substrate is then wound into a shape of a spiral cylinder to form the flexible heating assembly,
wherein the at least one heating circuit (12) is formed by magnetron sputtering coating.

2. The flexible heating assembly of claim 1, wherein the sheet-shaped flexible substrate (11) comprises at least one of aluminosilicate fiber paper, PI film, and casting ceramic sheet,
wherein the flexible protective film comprises at least one of casting sheet, nitride ceramic material, and oxide ceramic material, and
wherein the thermal expansion coefficient of the flexible protective film adapts to the thermal expansion coefficient of the sheet-shaped flexible substrate (11).

3. The flexible heating assembly of claim 1, wherein the flexible protective film comprises at least one of ZrO₂ composite film, Al₂O₃ composite film, SiO₂ composite film, and Si₃N₄ composite film prepared through direct current magnetron sputtering or radio frequency magnetron sputtering,
wherein the thickness of the flexible protective film is from 100 nm to 1000 nm, and
wherein the thickness of the at least one heating circuit (12) is from 1 µm to 3.5 µm, and the thickness of the conductive circuits (13) is from 1 µm to 5 µm.

4. The flexible heating assembly of claim 1, further comprising:
electrode leads (14) respectively connected to the conductive circuits (13).

5. The flexible heating assembly according to any of claims 1 to 4, wherein the at least one heating circuit (12) comprises a transition layer (121) disposed on the sheet-shaped flexible substrate (11) and a heating layer (122) disposed on the transition layer (121),
wherein the transition layer (121) comprises at least one of Cr, ZrNi, and TiN, and
wherein the heating layer (122) comprises at least one of Pt, AgPd, AuPd, PtRu, PtRh, NiCr, and NiCrAlY.

6. The flexible heating assembly according to any of claims 1 to 5, wherein the conductive circuits (13) comprise a bottom layer (131) disposed on the sheet-shaped flexible substrate (11), an intermediate buffer layer (132) disposed on the bottom layer (131), and a conductive layer (133) disposed on the intermediate buffer layer (132).

7. The flexible heating assembly of claim 6, wherein the bottom layer (131) comprises at least one of pure Ti, and pure Ni,
wherein the intermediate buffer layer (132) comprises at least one of pure Ti and pure Ni, and
wherein the conductive layer (133) comprises at least one of Au, Ag, and Cu.

8. A method for fabricating a flexible heating assembly, comprising:
a method for fabricating a flexible heating element, comprising;
S1: providing a sheet-shaped flexible substrate (11), and placing the sheet-shaped flexible substrate (11) into a coating machine cavity;
S2: performing magnetron sputtering on the sheet-shaped flexible substrate (11) to form at least one heating circuit (12);
S3: performing magnetron sputtering on the sheet-shaped flexible substrate (11) to form a conductive circuit (13); and
S4: performing magnetron sputtering on the at least one heating circuit (12) to form a protective film;
wherein the method for fabricating a flexible heating assembly further comprises coating an aerosol-generating substrate on the side surface of the heating element, on which the at least one heating circuit (12) is disposed, and then winding the heating element coated with the aerosol-generating substrate into a shape of a spiral cylinder to form the flexible heating assembly.

9. The method of claim 8, wherein the method further comprises:
in S1, wiping and cleaning the sheet-shaped flexible substrate (11) with alcohol,
placing the sheet-shaped flexible substrate (11) in a coating machine cavity,
vacuuming and preheating the coating machine cavity, and
ion-cleaning the surface of the sheet-shaped flexible substrate (11); and
in S4, introducing argon and oxygen in a ratio of 1:1 into the coating machine cavity until the working air pressure therein reaches 0.4 Pa;
turning on a first power supply for a SiO₂ target, a ZrO₂ target, an Al₂O₃ target, or a Si₃N₄ target; and
performing magnetron sputtering at a power density between 2 W/cm² and 6 W/cm² and at a temperature between room temperature and 500°C to form the protective film with a thickness between 100 nm and 1000 nm.

10. The method of claim 8, wherein S2 comprises:
performing magnetron sputtering on the sheet-shaped flexible substrate (11) to form a transition layer (121); and
performing magnetron sputtering on the transition layer (121) to form a heating layer (122).

11. The method of claim 10, wherein the method further comprises:
in S2, introducing argon into the coating machine cavity until the working air pressure therein reaches 0.5 Pa,
turning on a second power supply for a Cr target, a ZrNi target, or a TiN target,
coating a first film on the sheet-shaped flexible substrate (11) for 5 minutes to 15 minutes at a power density between 6 W/cm² and 8 W/cm² and at room temperature to form the transition layer (121) with a thickness between 10 nm and 200 nm, and
turning off the second power supply for the Cr target, the ZrNi target, or the TiN target,
turning on a third power supply for a NiCr target, a NiCrAlY target, a Pt target, an AgPd target, an AuPd target, a PtRu target, or a PtRh target, and
coating a second film on the transition layer (121) for 60 minutes to 120 minutes at a power density between 6 W/cm² and 8 W/cm² and at room temperature to form the heating layer (122) with a thickness between 1 µm and 2.5 µm.

12. The method of claim 8, wherein S3 comprises:
performing magnetron sputtering on the sheet-shaped flexible substrate (11) to form a bottom layer (131);
performing magnetron sputtering on the bottom layer (131) to form an intermediate buffer layer (132);
performing magnetron sputtering on the intermediate buffer layer (132) to form a conductive layer (133); and
soldering an electrode lead (14) on the conductive layer (133) to form a conductive electrode.

13. The method of claim 12, wherein the method further comprises:
in S3, introducing argon into the coating machine cavity until the working air pressure therein reaches 0.5 Pa,
turning on a fourth power supply for a Titanium target or a Nickel target,
coating a third film on the sheet-shaped flexible substrate (11) for 5 minutes to 10 minutes at a power density between 6 W/cm² and 8 W/cm² and at room temperature to form the bottom layer (131),
turning off the fourth power supply for the Titanium target or the Nickel target,
turning on a fifth power supply for a Nickel target or a Titanium target.
coating a fourth film (131) on the bottom layer for 10 minutes to 30 minutes at a power density between 6 W/cm² and 8 W/cm² and at room temperature to form the intermediate buffer layer (132),
turning off the fifth power supply for the Nickel target or the Titanium target,
turning on a sixth power supply for a silver target, a copper target, or a gold target,
and
coating a fifth film on the intermediate buffer layer (132) for 30 minutes to 120 minutes at a power density between 4 W/cm² and 8 W/cm² at room temperature to form the conductive layer (133).

## Patentansprüche

1. Biegsame Heizanordnung, umfassend:
ein Heizelement, welches umfasst:
ein plattenförmiges biegsames Substrat (11);
mindestens eine Heizschaltung (12);
leitfähige Schaltungen (13); und
einen biegsamen Schutzfilm;
wobei die mindestens eine Heizschaltung (12) auf dem plattenförmigen biegsamen Substrat (11) eingerichtet ist, die leitfähigen Schaltungen (13) auf dem plattenförmigen biegsamen Substrat (11) eingerichtet und jeweils mit den Enden der mindestens einen Heizschaltung (12) verbunden sind und der biegsame Schutzfilm die mindestens eine Heizschaltung (12) abdeckt; und
ein aerosolerzeugendes Substrat, das eine viskose Substanz umfasst;
wobei das aerosolerzeugende Substrat auf die Seitenoberfläche des Heizelements beschichtet ist, auf der die mindestens eine Heizschaltung (12) angeordnet ist, und das mit dem aerosolerzeugenden Substrat beschichtete Heizelement anschließend zu einer Form eines spiralförmigen Zylinders aufgewickelt wird, um die biegsame Heizanordnung zu bilden,
wobei die mindestens eine Heizschaltung (12) durch Magnetronsputterbeschichtung gebildet ist.

2. Biegsame Heizanordnung nach Anspruch 1, wobei das plattenförmige biegsame Substrat (11) mindestens eines von einem Aluminosilikatfaserpapier, einem PI-Film und einer Gusskeramikplatte umfasst,
wobei der biegsame Schutzfilm mindestens eines von einer Gussplatte, einem Nitridkeramikmaterial und einem Oxidkeramikmaterial umfasst und
wobei sich der Wärmeausdehnungskoeffizient des biegsamen Schutzfilms an den Wärmeausdehnungskoeffizienten des plattenförmigen biegsamen Substrats (11) anpasst.

3. Biegsame Heizanordnung nach Anspruch 1, wobei der biegsame Schutzfilm mindestens eines von einem ZrO₂-Verbundfilm, einem Al₂O₃-Verbundfilm, einem SiO₂-Verbundfilm und einem Si₃N₄-Verbundfilm, die durch Gleichstrom-Magnetronsputtern oder Hochfrequenz-Magnetronsputtern gefertigt sind, umfasst,
wobei die Dicke des biegsamen Schutzfilms von 100 nm bis 1000 nm beträgt und
wobei die Dicke der mindestens einen Heizschaltung (12) von 1 µm bis 3,5 µm beträgt und die Dicke der leitfähigen Schaltungen (13) von 1 µm bis 5 µm beträgt.

4. Biegsame Heizanordnung nach Anspruch 1, ferner umfassend:
Elektrodendrähte (14), die jeweils mit den leitfähigen Schaltungen (13) verbunden sind.

5. Biegsame Heizanordnung nach einem der Ansprüche 1 bis 4, wobei die mindestens eine Heizschaltung (12) eine auf dem plattenförmigen biegsamen Substrat (11) eingerichtete Übergangsschicht (121) und eine auf der Übergangsschicht (121) eingerichtete Heizschicht (122) umfasst,
wobei die Übergangsschicht (121) mindestens eines von Cr, ZrNi und TiN umfasst und
wobei die Heizschicht (122) mindestens eines von Pt, AgPd, AuPd, PtRu, PtRh, NiCr und NiCrAlY umfasst.

6. Biegsame Heizanordnung nach einem der Ansprüche 1 bis 5, wobei die leitfähigen Schaltungen (13) eine auf dem plattenförmigen biegsamen Substrat (11) eingerichtete untere Schicht (131), eine auf der unteren Schicht (131) eingerichtete Zwischenpufferschicht (132) und eine auf der Zwischenpufferschicht (132) eingerichtete leitfähige Schicht (133) umfassen.

7. Biegsame Heizanordnung nach Anspruch 6, wobei die untere Schicht (131) mindestens eines von reinem Ti und reinem Ni umfasst,
wobei die Zwischenpufferschicht (132) mindestens eines von reinem Ti und reinem Ni umfasst und
wobei die leitfähige Schicht (133) mindestens eines von Au, Ag und Cu umfasst.

8. Verfahren zum Herstellen einer biegsamen Heizanordnung, umfassend:
ein Verfahren zum Herstellen eines biegsamen Heizelements, umfassend;
S1: Bereitstellen eines plattenförmigen biegsamen Substrats (11) und Einlegen des plattenförmigen biegsamen Substrats (11) in einen Beschichtungsmaschinenhohlraum;
S2: Durchführen eines Magnetronsputterns auf dem plattenförmigen biegsamen Substrat (11), um mindestens eine Heizschaltung (12) zu bilden;
S3: Durchführen eines Magnetronsputterns auf dem plattenförmigen biegsamen Substrat (11), um eine leitfähige Schaltung (13) zu bilden; und
S4: Durchführen eines Magnetronsputterns auf der mindestens einen Heizschaltung (12), um einen Schutzfilm zu bilden;
wobei das Verfahren zum Herstellen einer biegsamen Heizanordnung ferner ein Beschichten eines aerosolerzeugenden Substrats auf die Seitenoberfläche des Heizelements, auf der die mindestens eine Heizschaltung (12) eingerichtet ist, und ein anschließendes Aufwickeln des mit dem aerosolerzeugenden Substrat beschichteten Heizelements zu einer Form eines spiralförmigen Zylinders umfasst, um die biegsame Heizanordnung zu bilden.

9. Verfahren nach Anspruch 8, wobei das Verfahren ferner Folgendes umfasst:
Abwischen und Reinigen des plattenförmigen biegsamen Substrats (11) mit Alkohol in S1,
Einlegen des plattenförmigen biegsamen Substrats (11) in einen Beschichtungsmaschinenhohlraum,
Absaugen und Vorheizen des Beschichtungsmaschinenhohlraums und Ionenreinigen der Oberfläche des plattenförmigen biegsamen Substrats (11); und
Einleiten von Argon und Sauerstoff in einem Verhältnis von 1:1 in den Beschichtungsmaschinenhohlraum in S4, bis der Arbeitsluftdruck darin 0,4 Pa erreicht;
Einschalten einer ersten Leistungsversorgung für ein SiO₂-Target, ein ZrO₂-Target, ein Al₂O₃-Target oder ein Si₃N₄-Target; und
Durchführen eines Magnetronsputterns bei einer Leistungsdichte zwischen 2 W/cm² und 6 W/cm² und bei einer Temperatur zwischen Raumtemperatur und 500 °C, um den Schutzfilm mit einer Dicke zwischen 100 nm und 1000 nm zu bilden.

10. Verfahren nach Anspruch 8, wobei S2 Folgendes umfasst:
Durchführen eines Magnetronsputterns auf dem plattenförmigen biegsamen Substrat (11), um eine Übergangsschicht (121) zu bilden; und
Durchführen eines Magnetronsputterns auf der Übergangsschicht (121), um eine Heizschicht (122) zu bilden.

11. Verfahren nach Anspruch 10, wobei das Verfahren ferner Folgendes umfasst:
Einleiten von Argon in den Beschichtungsmaschinenhohlraum in S2, bis der Arbeitsluftdruck darin 0,5 Pa erreicht,
Einschalten einer zweiten Leistungsversorgung für ein Cr-Target, ein ZrNi-Target oder ein TiN-Target,
Beschichten eines ersten Films auf das plattenförmige biegsame Substrat (11) 5 Minuten bis 15 Minuten lang bei einer Leistungsdichte zwischen 6 W/cm² und 8 W/cm² und bei Raumtemperatur, um die Übergangsschicht (121) mit einer Dicke zwischen 10 nm und 200 nm zu bilden, und
Abschalten der zweiten Leistungsversorgung für das Cr-Target, das ZrNi-Target oder das TiN-Target,
Einschalten einer dritten Leistungsversorgung für ein NiCr-Target, ein NiCrAlY-Target, ein Pt-Target, ein AgPd-Target, ein AuPd-Target, ein PtRu-Target oder ein PtRh-Target und
Beschichten eines zweiten Films auf die Übergangsschicht (121) 60 Minuten bis 120 Minuten lang bei einer Leistungsdichte zwischen 6 W/cm² und 8 W/cm² und bei Raumtemperatur, um die Heizschicht (122) mit einer Dicke zwischen 1 µm und 2,5 µm zu bilden.

12. Verfahren nach Anspruch 8, wobei S3 Folgendes umfasst:
Durchführen eines Magnetronsputterns auf dem plattenförmigen biegsamen Substrat (11), um eine untere Schicht (131) zu bilden;
Durchführen eines Magnetronsputterns auf der unteren Schicht (131), um eine Zwischenpufferschicht (132) zu bilden;
Durchführen eines Magnetronsputterns auf der Zwischenpufferschicht (132), um eine leitfähige Schicht (133) zu bilden; und
Löten eines Elektrodendrahtes (14) auf die leitfähige Schicht (133), um eine leitfähige Elektrode zu bilden.

13. Verfahren nach Anspruch 12, wobei das Verfahren ferner Folgendes umfasst:
Einleiten von Argon in den Beschichtungsmaschinenhohlraum in S3, bis der Arbeitsluftdruck darin 0,5 Pa erreicht,
Einschalten einer vierten Leistungsversorgung für ein Titan-Target oder ein Nickel-Target,
Beschichten eines dritten Films auf das plattenförmige biegsame Substrat (11) 5 Minuten bis 10 Minuten lang bei einer Leistungsdichte zwischen 6 W/cm² und 8 W/cm² und bei Raumtemperatur, um die untere Schicht (131) zu bilden,
Abschalten der vierten Leistungsversorgung für das Titan-Target oder das Nickel-Target,
Einschalten einer fünften Leistungsversorgung für ein Nickel-Target oder ein Titan-Target.
Beschichten eines vierten Films (131) auf die untere Schicht 10 Minuten bis 30 Minuten lang bei einer Leistungsdichte zwischen 6 W/cm² und 8 W/cm² und bei Raumtemperatur, um die Zwischenpufferschicht (132) zu bilden,
Abschalten der fünften Leistungsversorgung für das Nickel-Target oder das Titan-Target,
Einschalten einer sechsten Leistungsversorgung für ein Silber-Target, ein Kupfer-Target oder ein Gold-Target und
Beschichten eines fünften Films auf die Zwischenpufferschicht (132) 30 Minuten bis 120 Minuten lang bei einer Leistungsdichte zwischen 4 W/cm² und 8 W/cm² bei Raumtemperatur, um die leitfähige Schicht (133) zu bilden.

## Revendications

1. Ensemble chauffant flexible, comprenant :
un élément chauffant, comprenant :
un substrat flexible en forme de feuille (11) ;
au moins un circuit chauffant (12) ;
des circuits conducteurs (13) ; et
un film protecteur flexible ;
dans lequel le ou les circuits chauffants (12) sont disposés sur le substrat flexible en forme de feuille (11), les circuits conducteurs (13) sont disposés sur le substrat flexible en forme de feuille (11) et respectivement connectés aux extrémités du ou des circuits chauffants (12), et le film protecteur flexible recouvre le ou les circuits chauffants (12) ; et
un substrat générateur d'aérosol comprenant une substance visqueuse ;
dans lequel le substrat générateur d'aérosol est revêtu sur la surface latérale de l'élément chauffant, sur lequel sont disposés le ou les circuits chauffants (12), et l'élément chauffant revêtu du substrat générateur d'aérosol est ensuite enroulé en forme de cylindre spiralé pour former l'ensemble chauffant flexible,
dans lequel les ou les circuits chauffants (12) sont formés par revêtement par pulvérisation magnétronique.

2. Ensemble chauffant flexible selon la revendication 1, dans lequel le substrat flexible en forme de feuille (11) comprend au moins l'un de papier de fibres d'aluminosilicate, de film PI et d'une feuille de céramique coulée,
dans lequel le film protecteur flexible comprend au moins l'un d'une feuille de coulée, d'un matériau céramique nitruré et d'un matériau céramique oxyde, et
dans lequel le coefficient de dilatation thermique du film protecteur flexible s'adapte au coefficient de dilatation thermique du substrat flexible en forme de feuille (11).

3. Ensemble chauffant flexible selon la revendication 1, dans lequel le film protecteur flexible comprend au moins l'un d'un film composite de ZrO₂, d'un film composite d'Al₂O₃, d'un film composite de SiO₂ et d'un film composite de Si₃N₄ préparé par pulvérisation magnétronique à courant continu ou par pulvérisation magnétronique à radiofréquence,
dans lequel l'épaisseur du film protecteur flexible est comprise entre 100 nm et 1000 nm, et
dans lequel l'épaisseur du ou des circuits chauffants (12) est de 1 µm à 3,5 µm et l'épaisseur des circuits conducteurs (13) est de 1 µm à 5 µm.

4. Ensemble chauffant flexible selon la revendication 1, comprenant en outre :
des conducteurs d'électrodes (14) respectivement connectés aux circuits conducteurs (13).

5. Ensemble chauffant flexible selon l'une quelconque des revendications 1 à 4, dans lequel le ou les circuits chauffants (12) comprennent une couche de transition (121) disposée sur le substrat flexible en forme de feuille (11) et une couche chauffante (122) disposée sur la couche de transition (121),
dans lequel la couche de transition (121) comprend au moins l'un de : Cr, ZrNi et TiN, et
dans lequel la couche chauffante (122) comprend au moins l'un de : Pt, AgPd, AuPd, PtRu, PtRh, NiCr et NiCrAlY.

6. Ensemble chauffant flexible selon l'une quelconque des revendications 1 à 5, dans lequel les circuits conducteurs (13) comprennent une couche inférieure (131) disposée sur le substrat flexible en forme de feuille (11), une couche tampon intermédiaire (132) disposée sur la couche inférieure (131) et une couche conductrice (133) disposée sur la couche tampon intermédiaire (132).

7. Ensemble chauffant flexible selon la revendication 6, dans lequel la couche inférieure (131) comprend au moins l'un de Ti pur et de Ni pur,
dans lequel la couche tampon intermédiaire (132) comprend au moins l'un de Ti pur et de Ni pur, et
dans lequel la couche conductrice (133) comprend au moins l'un de : Au, Ag et Cu.

8. Procédé de fabrication d'un ensemble chauffant flexible, comprenant :
un procédé de fabrication d'un élément chauffant flexible, comprenant ;
S1 : la fourniture d'un substrat flexible en forme de feuille (11) et le placement du substrat flexible en forme de feuille (11) dans une cavité de machine à revêtement ;
S2 : la réalisation d'une pulvérisation magnétronique sur le substrat flexible en forme de feuille (11) pour former au moins un circuit chauffant (12) ;
S3 : la réalisation d'une pulvérisation magnétronique sur le substrat flexible en forme de feuille (11) pour former un circuit conducteur (13) ; et
S4 : la réalisation d'une pulvérisation magnétronique sur le ou les circuits chauffants (12) pour former un film protecteur ;
dans lequel le procédé de fabrication d'un ensemble chauffant flexible comprend en outre le revêtement d'un substrat générateur d'aérosol sur la surface latérale de l'élément chauffant, sur lequel sont disposés le ou les circuits chauffants (12), puis l'enroulement de l'élément chauffant revêtu du substrat générateur d'aérosol en forme de cylindre spiralé pour former l'ensemble chauffant flexible.

9. Procédé selon la revendication 8, dans lequel le procédé comprend en outre :
en S1, l'essuyage et le nettoyage du substrat flexible en forme de feuille (11) avec de l'alcool,
le placement du substrat flexible en forme de feuille (11) dans une cavité de machine à revêtement,
la mise sous vide et le préchauffage de la cavité de machine à revêtement, et
le nettoyage ionique de la surface du substrat flexible en forme de feuille (11) ; et
en S4, l'introduction d'argon et d'oxygène dans un rapport de 1:1 dans la cavité de machine à revêtement jusqu'à ce qu'une pression d'air de travail à l'intérieur atteigne 0,4 Pa ;
la mise en marche d'une première alimentation en puissance pour une cible de SiO₂, une cible de ZrO₂, une cible d'Al₂O₃ ou une cible de Si₃N₄ ; et
la réalisation d'une pulvérisation magnétronique à une densité de puissance comprise entre 2 W/cm² et 6 W/cm² et à une température comprise entre la température ambiante et 500 °C pour former le film protecteur d'une épaisseur comprise entre 100 nm et 1000 nm.

10. Procédé selon la revendication 8, dans lequel S2 comprend :
la réalisation d'une pulvérisation magnétronique sur le substrat flexible en forme de feuille (11) pour former une couche de transition (121) ; et
la réalisation d'une pulvérisation magnétronique sur la couche de transition (121) pour former une couche chauffante (122).

11. Procédé de la revendication 10, dans lequel le procédé comprend en outre :
en S2, l'introduction d'argon dans la cavité de machine à revêtement jusqu'à ce qu'une pression d'air de travail à l'intérieur atteigne 0,5 Pa,
la mise en marche d'une deuxième alimentation en puissance pour une cible de Cr, une cible de ZrNi ou une cible de TiN,
le revêtement d'un premier film sur le substrat flexible en forme de feuille (11) pendant 5 minutes à 15 minutes à une densité de puissance comprise entre 6 W/cm² et 8 W/cm² et à température ambiante pour former la couche de transition (121) d'une épaisseur comprise entre 10 nm et 200 nm, et
l'arrêt de la deuxième alimentation en puissance pour la cible de Cr, la cible de ZrNi ou la cible de TiN,
la mise en marche d'une troisième alimentation en puissance pour une cible de NiCr, une cible de NiCrAlY, une cible de Pt, une cible d'AgPd, une cible d'AuPd, une cible de PtRu ou une cible et PtRh, et
le revêtement d'un second film sur la couche de transition (121) pendant 60 minutes à 120 minutes à une densité de puissance comprise entre 6 W/cm² et 8 W/cm² et à température ambiante pour former la couche chauffante (122) d'une épaisseur comprise entre 1 µm et 2,5 µm.

12. Procédé selon la revendication 8, dans lequel S3 comprend :
la réalisation d'une pulvérisation magnétronique sur le substrat flexible en forme de feuille (11) pour former une couche inférieure (131) ;
la réalisation d'une pulvérisation magnétronique sur la couche inférieure (131) pour former une couche tampon intermédiaire (132) ;
la réalisation d'une pulvérisation magnétronique sur la couche tampon intermédiaire (132) pour former une couche conductrice (133) ; et
le soudage d'un fil d'électrode (14) sur la couche conductrice (133) pour former une électrode conductrice.

13. Procédé selon la revendication 12, dans lequel le procédé comprend en outre :
en S3, l'introduction d'argon dans la cavité de machine à revêtement jusqu'à ce qu'une pression d'air de travail à l'intérieur atteigne 0,5 Pa,
la mise en marche d'une quatrième alimentation en puissance pour une cible de titane ou une cible de nickel,
le revêtement d'un troisième film sur le substrat flexible en forme de feuille (11) pendant 5 minutes à 10 minutes à une densité de puissance comprise entre 6 W/cm² et 8 W/cm² et à température ambiante pour former la couche inférieure (131),
l'arrêt de la quatrième alimentation en puissance pour la cible de titane ou la cible de nickel,
la mise en marche d'une cinquième alimentation en puissance pour une cible de nickel ou une cible de titane,
le revêtement d'un quatrième film (131) sur la couche inférieure pendant 10 minutes à 30 minutes à une densité de puissance comprise entre 6 W/cm² et 8 W/cm² et à température ambiante pour former la couche tampon intermédiaire (132),
l'arrêt de la cinquième alimentation en puissance pour la cible de nickel ou la cible de titane,
la mise en marche d'une sixième alimentation en puissance pour une cible d'argent, une cible de cuivre ou une cible d'or, et
le revêtement d'un cinquième film sur la couche tampon intermédiaire (132) pendant 30 minutes à 120 minutes à une densité de puissance comprise entre 4 W/cm² et 8 W/cm² à température ambiante pour former la couche conductrice (133).
